

June 15, 1954

C. O. TONGBERG ET AL  
LUBRICATING OIL COMPOSITION

2,681,315

Filed Sept. 4, 1951



Carl O. Tongberg Inventors  
William H. Brugmann, Jr.

By *John M. Thomas* Attorney

## UNITED STATES PATENT OFFICE

2,681,315

## LUBRICATING OIL COMPOSITION

Carl O. Tongberg, Westfield, and William H. Brugmann, Jr., Elizabeth, N. J., assignors to Standard Oil Development Company, a corporation of Delaware

Application September 4, 1951, Serial No. 245,058

14 Claims. (Cl. 252—33.4)

1

The present invention relates to a composition comprising a major portion of a lubricating oil and minor portions of rust preventive and detergent additives.

It is known to the art to employ oil-soluble petroleum sulfonates and oil-miscible alkaryl polyether alcohols in combination in lubricants to render the oil relatively non-corrosive to metal parts. Such a composition affords protection under certain conditions against corrosion or rusting by moisture and aqueous solutions of electrolytes. It is frequently desired to use oil-soluble calcium petroleum sulfonates in oils since they are extremely effective as engine oil detergent additives; however, calcium sulfonates, used in combination with a polyether alcohol, do not give the desired degree of protection from rusting required in certain types of oils. In addition, calcium petroleum sulfonates and alkaryl polyether alcohols are not always compatible with one another. Haze formation occurs in many cases when these particular additives are employed in combination, and the haze does not disappear even upon prolonged standing.

It is also known in the art to compound oils with small amounts of a metal salt of an alkyl phenol sulfide and an oil soluble salt of a petroleum sulfonate to prepare lubricating compositions having desired detergent and non-corrosive properties. Such compositions, however, do not give the desired protection from moisture corrosion for certain types of uses.

It has been found that unexpectedly improved anti-rusting properties are imparted to a lubricating oil, preferably a mineral oil, by compounding with it at least three different components, each component being added in relatively small amounts. These components include a water-insoluble, oil-miscible alkaryl polyether alcohol, an oil-soluble calcium petroleum sulfonate, and an alkaline earth metal salt of an alkyl phenol sulfide.

The alkaryl polyether alcohol is an alkylphenoxypolyethoxyethanol having from two to six ether groups. Preferred compounds of this class are illustrated by the formula:



wherein R and R' are selected from the class consisting of hydrogen and alkyl radicals having 4 to 12 carbon atoms, x is 1 to 5, and the polyethoxy radical is straight chain. The alkyl radicals

should be of sufficient size and number to impart oil solubility to the compound and may be butyl, amyl, hexyl, octyl, nonyl, dodecyl and the like, either the straight or branched chain configurations being useful. The phenoxy radical preferably has no more than two alkyl groups. When the aryl radical has only one alkyl group, it may be positioned in the ortho, meta- or para-position with respect to the polyether group. An octyl radical, particularly a tertiary radical, such as that derived by alkylation with diisobutylene, is very effective in the practice of the present invention. Preferably, the alcohol derivative contains five ether groups and only one alkyl group.

The polyether alcohols are conveniently prepared by methods known in the art. An alkylated phenol is reacted with from two to six mols of ethylene oxide in one method of preparation. In another, it is convenient to react the alkylated phenol with an alkyl halohydrin such as triethylene halohydrin in the presence of a base.

The polyether alcohol may be used in the composition in concentrations as low as about 0.05%, preferably above 0.1 weight per cent, and up to the limit of the solubility of the compound in the oil being used. The size and number of alkyl groups in the polyether alcohol will determine to a large extent the solubility of the compound in the composition. Generally the upper limit of solubility will be in the order of about 3 to 4%. A preferred range will be from about 0.2 to 2% by weight of the polyether alcohol based on the total composition.

The oil-soluble calcium petroleum sulfonates used in the present invention are the salts of oil-soluble or so-called "mahogany" acids. They may be prepared by neutralizing acid treated oils or extracted sulfonic acids directly with a stoichiometric amount of calcium oxide or hydroxide. However, it is often more convenient to prepare them from the sodium salts by double decomposition. Particularly advantageous also are calcium petroleum sulfonates having an excess rather than a stoichiometric amount of calcium added to the sulfonic acid. Calcium sulfonates having an excess of calcium may be prepared by the procedure described in U. S. Patent No. 2,467,176 to Zimmer, Carlson and Duncan. The term "oil-soluble calcium petroleum sulfonates," as used in the present specification and claims, refers to both of the above general types of calcium sulfonates.

The molecular weight of the calcium sulfonates may vary from about 750 to as high as 1100, al-

though as a general rule it is preferred that the sulfonates have a molecular weight in the range of 800 to 1000. The sulfonates may be used in the finished composition in amounts ranging from about 0.4 to as high as 10.0 weight per cent on a dry basis. Preferably, the sulfonates may be used in amounts ranging from 0.5 to 5% by weight based on the total composition and in many cases amounts of from 0.5 to 2% will be entirely adequate to impart the desired detergency characteristics to the finished oil and to cooperate with the other additives in improving the anti-corrosive properties of the oil.

The alkaline earth metal salts of alkyl phenol sulfides are well known as being effective detergents and sludge dispersers for lubricating oils. For example, the preparation of calcium salts of this type, and their use in lubricants, is described in the Mikeska patent U. S. 2,362,289. The preparation of barium salts is described in the Winning patent, U. S. 2,362,291. The magnesium salts are described in the McNab patent, U. S. 2,362,292, and mixed alkaline earth salts containing two different alkaline earth metals are described and claimed in U. S. 2,480,664 to McNab, McNulty and Cross.

In the present invention, the alkaline earth metal salts of alkylated phenol sulfides have at least one alkyl group attached to each benzene nucleus. The alkaline earth metals include calcium, barium, strontium, and magnesium. The presence of at least one alkyl group in the benzene nucleus is necessary to impart oil solubility to the compound. The alkyl groups should contain at least 4 carbon atoms each and preferably

4 content sulfides known to the art. The phenol sulfide salts are used in amounts ranging from about 0.2 to 10.0 weight per cent based on the total composition. Amounts in the range of 0.5 to 5.0 weight per cent are generally preferred.

5 As a general rule, it is preferred that the weight ratio of the alkaline earth metal alkyl phenol sulfide to calcium sulfonates be in the range of 0.1 to 3.5 to obtain effective corrosion prevention properties.

10 The following examples will illustrate the advantages of the present invention.

#### EXAMPLE 1

15 A series of blends were prepared employing as base stock an SAE 30 grade motor oil derived from a solvent extracted Mid-Continent crude fraction. The blends included as additives tert-octyl phenyl ether alcohol having 5 ether groups<sup>1</sup> (additive 1) alone and in combination with either 20 barium tert-octyl phenol sulfide (additive 2) or calcium petroleum sulfonates having an average molecular weight of about 950. Other blends included combinations of additive 2 and calcium petroleum sulfonate and of these materials with additive 1.

25 The blends were tested by coating standard steel panels with the oil and placing the panels in a standard humidity cabinet maintained at a temperature of 100° F., and a relative humidity of 100%. The time in hours required to rust the panels in the cabinet is termed the humidity cabinet life. The tendency of the blends to form haze was also noted. Results of tests are shown in Table I below:

Table I.—Additives used in SAE 30 base stock

| Blend No. | Additive 2 (Wt. Percent) | Calcium Sulfonate (Wt. Percent) | Wt. Ratio, Additive 2 to Calcium Sulfonate | Additive 1 (Wt. Percent) | Haze Formation | Humidity Cabinet Life (Hrs.) |
|-----------|--------------------------|---------------------------------|--------------------------------------------|--------------------------|----------------|------------------------------|
| 1         | 0                        | 0                               | —                                          | 0.5                      | No             | 0                            |
| 2         | 1.38                     | 0                               | —                                          | 0.5                      | No             | ≤3                           |
| 3         | 0                        | 0.618                           | 0                                          | 0.5                      | Yes            | <48                          |
| 4         | 0                        | 0.618                           | 0                                          | 0.5                      | Yes            | —                            |
| 5         | 1.38                     | 0.618                           | 2.22                                       | 0                        | No             | <3                           |
| 6         | 0.55                     | 1.241                           | 0.44                                       | 0.5                      | No             | 288                          |
| 7         | 1.10                     | 0.823                           | 1.34                                       | 0.5                      | No             | >288                         |
| 8         | 1.38                     | 0.618                           | 2.22                                       | 0.5                      | No             | 288                          |
| 9         | 1.38                     | 0.618                           | 2.22                                       | 0.5                      | No             | 240                          |
| 10        | 1.38                     | 0.618                           | 2.22                                       | 0.6                      | No             | 264                          |
| 11        | 1.66                     | 0.413                           | 4.00                                       | 0.5                      | No             | 168                          |

should contain from 4 to 12 or more carbon atoms. The alkyl radicals may be straight chain or branched. The scope of the invention is not limited as to the number of sulfur atoms which interconnect the benzene nucleus, but compounds containing from 1 to 4 sulfur atoms in such linkage are preferred. The sulfide may contain only one alkaline earth metal, or may include a mixture of two alkaline earth metals. Barium is the preferred metal when the sulfide contains only one alkaline earth metal, but it is preferred in the case of mixed salts to employ calcium and barium.

The phenol sulfide salt may be prepared by procedures well known to the art in which the equivalent of one mol of the desired metal base is used for each pair of phenol radicals. If desired, at least one mol of the metal compound may be used for each mol of phenol radical to produce an additive having a high content of the alkaline earth metal. The term "alkaline earth metal salt of an alkyl phenol sulfide" as used herein refers broadly to the single and mixed salts of the phenol sulfide and to the high metal-

55 Additive 1 alone or in combination with either calcium sulfonate or additive 2 gave substantially no or only fair protection in the humidity cabinet test when using relatively low concentrations of the additives. The combination of calcium sulfonate and additive 2 likewise gives no protection. However, by combining all three additives, an unexpected increase in humidity cabinet 60 life was realized. Indeed, a synergistic effect is achieved since the relatively good cabinet life of the blend containing calcium sulfonate and alkaryl polyether alcohol is increased over five times by addition of a small amount of barium tert-octyl phenol sulfide, a compound which even in combination with the alkaryl polyether alcohol gives no particular rust protection in a humidity cabinet as indicated by blend 2. A haze 65 resulted in the oil when using only calcium sulfonate and polyether alcohol (blends 3 and 4) which did not disappear even after standing for one week. No haze formation occurred when

the barium tert-octyl phenol sulfide was used with the other two additives.

The relations between weight ratio of additive 2 to calcium sulfonates and humidity cabinet life for the blends containing 0.5 weight per cent of the polyether alcohol are shown in the graph in Fig. 1 of the accompanying drawing. Blends having a humidity cabinet life above about 190 to 200 hours were obtained at weight ratios in the range of about 0.1 to 3.5. Generally, it is preferred that the concentration of calcium sulfonates be above about 0.5 weight per cent of the total blend in order to obtain the desired protection against moisture corrosion.

#### EXAMPLE 2

A series of blends similar to those made in Example 1 were prepared by using an SAE 30 base oil, and a mixed calcium-barium salt of tert-octyl phenol sulfide (additive 3) was used in place of the barium salt. The salt contained about 75 wt. per cent calcium and 25 wt. per cent barium based on the total metal content of the compound. The calcium sulfonate and alkaryl polyether alcohol (additive 1) used in these blends were identical to those used in Example 1. Results are shown in Table II:

Table II.—Additives used in SAE base stock

| Blend No. | Additive 3 (Wt. Percent) | Calcium Sulfonate (Wt. Percent) | Wt. Ratio, Additive 3 to Calcium Sulfonate | Additive 1 (Wt. Percent) | Humidity Cabinet Life, Hrs. |
|-----------|--------------------------|---------------------------------|--------------------------------------------|--------------------------|-----------------------------|
| 12-----   | 0.66                     | 0.825                           | 0.8                                        | 0                        | 24-48                       |
| 13-----   | 1.00                     | 0.705                           | 1.42                                       | 0                        | 168                         |
| 14-----   | 1.00                     | 0.705                           | 1.42                                       | 0.5                      | 288                         |

A combination of the mixed metal phenol sulfide (additive 3) and calcium sulfonates in different ratios gave some protection, but, by adding a small amount of additive 1, the humidity cabinet life was increased very appreciably.

#### EXAMPLE 3

A series of blends were prepared in the same manner as those prepared in Example 1 using additive 2 and calcium petroleum sulfonate and, in place of additive 1, an alkaryl polyether alcohol having 3 ether groups (tert-octyl phenoxyethoxyethoxyethanol) termed (additive 4). Humidity cabinet life was then determined as shown below:

Table III.—Additives used in SAE 30 base stock

| Blend No. | Additive 2 (Wt. Percent) | Calcium Sulfonate (Wt. Percent) | Wt. Ratio, Additive 2 to Calcium Sulfonate | Additive 4 (Wt. Percent) | Humidity Cabinet Life, Hrs. |
|-----------|--------------------------|---------------------------------|--------------------------------------------|--------------------------|-----------------------------|
| 15-----   | 0.55                     | 1.24                            | 0.44                                       | 0.5                      | 288                         |
| 16-----   | 1.10                     | 0.83                            | 1.33                                       | 0.5                      | >288                        |
| 17-----   | 1.65                     | 0.41                            | 4.03                                       | 0.5                      | 168                         |

It is seen that alkaryl polyether alcohols having three ether groups have substantially the same potency in rust inhibition as those with five ether groups.

#### EXAMPLE 4

Two different SAE 30 grade motor oils were blended in each case with 0.5 weight per cent of additive 1 (Example 1) and 1.05 weight per cent of calcium petroleum sulfonate. In one case, where the oil was derived from a conventionally phenol solvent extracted Mid-Continent

lubricant fraction, considerable haze was formed which did not disappear after standing for one week at room temperature. In the other case, with an oil derived from a conventionally propane and cresylic acid solvent extracted Mid-Continent fraction slight haze formation occurred. In both cases, haze disappeared only after adding a small amount of metal phenol sulfide. It is seen that the extent of haze formation will vary depending on the type and treatment of the base oil.

The lubricating oil base stocks used in the compositions of this invention may be straight mineral lubricating oils or distillates derived from paraffinic, naphthenic, asphaltic or mixed base crudes, or if desired, various blended oils may be employed as well as residuals, particularly those from which asphaltic constituents have been carefully removed. Hydrogenated oils or white oils may be employed as well as synthetic oils prepared, for example, by the polymerization of olefins or by the reaction of oxides of carbon with hydrogen or by the hydrogenation of coal or its products. In certain instances cracking coil tar fractions and coal tar or shale oil distillates may also be used. Also for special ap-

plications, animal, vegetable or fish oils or their hydrogenated or volatilized products may be employed, either alone or in admixture with mineral oils.

The lubricating oils may vary considerably in viscosity and other properties depending upon the particular use for which they are desired, but they usually range from about 40 to 150 seconds Saybolt viscosity at 210° F. For the lubrication of certain low and medium speed diesel engines, the general practice has often been to use a lubricating oil base stock prepared from naphthenic or aromatic crudes and having a Saybolt viscosity at 210° F. of 45 to 90 seconds

and a viscosity index of 0 to 50. However, in certain types of diesel service, particularly with high speed diesel engines, and in aviation engine and other gasoline engine service, oils of higher viscosity index are often preferred, for example up to 75 to 100, or even higher viscosity index.

In addition to the materials to be added according to the present invention, other agents may also be used such as dyes, pour depressors, heat thickened fatty oils, sulfurized fatty oils, anti-oxidants, thickeners, viscosity index im-

provers, oiliness agents, resins, rubber, olefin polymers, voltolized fats, voltolized mineral oils, and/or voltolized waxes and colloidal solids such as graphite or zinc oxide, etc.

What is claimed is:

1. A composition of matter comprising a major amount of a mineral lubricating oil and, based on total composition, about 0.4 to 10% by weight of calcium petroleum sulfonate, about 0.05 to 4% by weight of an oil miscible alkylphenoxypolyethoxyethanol having from two to six ether groups, and 0.2 to 10% by weight of an alkaline earth metal salt of an alkyl phenol sulfide.
2. A composition of matter comprising a major amount, based on total composition, of a mineral lubricating oil and rust-inhibiting amounts of about 0.4 to 10% by weight of an oil-soluble calcium petroleum sulfonate, about 0.2 to 10% by weight of an alkaline earth metal salt of an alkyl phenol sulfide, and about 0.05 to 4% by weight of an alkaryl polyether alcohol having the formula:



wherein R and R' are selected from the group consisting of hydrogen and alkyl radicals having 4 to 12 carbon atoms and at least one R is an alkyl radical and x is from 1 to 5.

3. Composition in accordance with claim 2 in which said sulfonate has a molecular weight in the range of 750 to 1100.

4. A composition comprising a major proportion of a mineral lubricating oil and, based on total composition, about 0.4 to 10% by weight of an oil-soluble calcium petroleum sulfonate, about 0.05 to 4% by weight of an alkylphenoxypolyethoxyethanol having one alkyl group of 4 to 12 carbon atoms and from 1 to 5 ethoxy groups, and about 0.2 to 10% by weight of an alkaline earth metal salt of an alkyl phenol sulfide, said sulfide and sulfonate being present in a weight ratio in the range of 0.1 to 3.5.

5. A composition in accordance with claim 4 in which said alkyl group is tert.-octyl.

6. A lubricant comprising a major proportion of a mineral lubricating oil and 0.4 to 10% of an oil-soluble calcium petroleum sulfonate, 0.1 to 3.0% of an oil-soluble alkylphenoxypolyethoxyethanol having from 1 to 5 ethoxy groups, and from 0.2 to 10% of a salt of an alkyl phenol

sulfide containing at least one alkaline earth metal.

7. A non-rusting, haze-free lubricant composition comprising essentially a major proportion of a mineral lubricating oil and 0.5 to 5% of an oil-soluble calcium petroleum sulfonate having a molecular weight in the range of 750 to 1100, from 0.5 to 5% of an alkaline earth metal salt of an alkyl phenol sulfide, and from 0.2 to 2.0% of a compound having the formula:



wherein R and R' are selected from the group consisting of hydrogen and alkyl radicals having 4 to 12 carbon atoms and at least one R is an alkyl radical and x is from 2 to 4.

8. A composition in accordance with claim 7 in which said alkyl radical is tert.-octyl.

9. A composition in accordance with claim 7 in which said alkaline earth metal is barium.

10. A composition in accordance with claim 7 in which said alkaline earth metal is calcium.

11. A composition in accordance with claim 7 in which said alkaline earth metal is a mixture of calcium and barium.

12. A composition in accordance with claim 7 in which the weight ratio of said alkyl phenol sulfide salt to said calcium sulfonate is in the range of 0.1 to 3.5.

13. A composition in accordance with claim 7 in which said alkyl phenol sulfide is barium tert.-octyl phenol sulfide.

14. A composition in accordance with claim 7 in which said alkyl phenol sulfide is a mixed calcium and barium salt of tert.-octyl phenol sulfide.

40 References Cited in the file of this patent  
UNITED STATES PATENTS

| Number       | Name           | Date          |
|--------------|----------------|---------------|
| 2,361,804    | Wilson         | Oct. 31, 1944 |
| 45 2,366,191 | Jenkins        | Jan. 2, 1945  |
| 2,398,416    | Denison et al. | Apr. 16, 1946 |
| 2,447,607    | Zimmer et al.  | Aug. 24, 1948 |
| 2,485,150    | Glavis et al.  | Oct. 18, 1949 |
| 2,485,376    | Glavis et al.  | Oct. 18, 1949 |

## FOREIGN PATENTS

| Number     | Country       | Date          |
|------------|---------------|---------------|
| 50 616,381 | Great Britain | Jan. 28, 1949 |